

## UNITED STATES PATENT OFFICE

1,966,755

## PROCESS OF PREPARING DIAZO-TYPES

Guy Grandsaignes D'Hauterive, St.-Denis, France,  
assignor to Kalle & Co. Aktiengesellschaft,  
Wiesbaden-Biebrich, Germany

No Drawing. Application November 4, 1932,  
Serial No. 641,321. In France November 9,  
1931

6 Claims. (Cl. 95—6)

Photographic papers are known whose light-sensitive layer chiefly consists of a light-sensitive diazo compound. These known papers, after exposure to light under a pattern, yield pictures, if they are treated under suitable conditions with a solution of an azo component. This process of treating the pictures with a liquid developer involves, however, a great drawback in comparison with certain other papers which permit the production of pictures by the simple action of ammonia gas without the aid of any liquid.

The present invention relates to a process of preparing diazo-types. It comprises subjecting a material sensitized by means of a light sensitive aromatic diazo compound to light under a pattern or design and then causing the vapors of an aromatic amine, which is volatile to a certain degree and capable of coupling with diazo compounds, to act upon the material thus treated. According to this method a dyestuff is formed at those portions of the sensitive material which were not exposed to light. Thus a positive dyestuff picture is obtained from a positive design and vice versa. The after treatment with the aromatic amine can be carried out in different ways. The amine may be vaporized and the vapors thus obtained act upon the exposed material. Or, the amine is dissolved in a suitable solvent, for instance alcohol, and a support, such as blotting paper, paper, tissue or the like is impregnated with this solution and, after evaporation of the solvent, brought in contact with the exposed material. Thereby, vapors of the amine rise from the impregnated support and act upon those portions of the diazo compound in the sensitive material which have not been destroyed by light.

The process according to this invention has the following advantages:

- 40 1. It permits the preparation in a simple manner of the light-sensitive layer which, in principle, does not contain more than one diazo compound.
- 45 2. For the development there are used gaseous products which have not the odor of ammonia gas, since certain amines which can be utilized according to the process of this invention evolve practically odorless vapors.

50 3. The pictures can be developed by means of a simple apparatus, which does not take much room and is quite economic, as it will be described more in detail below.

This process may be applied to light-sensitive material of any kind, for instance to paper, films, 55 plates or the like.

For preparing light-sensitive papers one of the following processes may, for instance, be utilized: On the paper there is applied a layer of a solution of the diazo compound in water or in a suitable more or less aqueous organic solvent and the 60 excess of liquid is removed, for instance by means of a doctor device, as it is usually done in the preparation of the so-called ferrocyanide papers; or, on the surface of the suitably pretreated paper there is applied a layer of a colloidal solution, for instance collodion, or a more or less aqueous gelatine solution, in which the light-sensitive diazo compound has been dissolved.

For the production of light-sensitive films for the process of the present invention one proceeds 70 as follows: The film mass is impregnated with a solution of a diazo compound in a solvent which is capable of penetrating into the film mass; or there is applied on the film a solution of the diazo compound in a solvent, which vaporizes rapidly, 75 but at the same time rapidly penetrates into the film; or there is applied on the film a colloidal solution, for instance collodion, or a more or less aqueous gelatine solution in which the light-sensitive diazo compound has been dissolved: or there 80 is vaporized on a provisional support, for instance on a metal strap, a colloidal solution, for instance collodion, or a solution of methylcellulose, in which the light-sensitive diazo compound has been dissolved.

85 It is also possible to add to the light-sensitive diazo compound bodies, such as metal salts, which are capable of altering the shade of the dyestuffs obtained by the development or of forming with these dyestuffs insoluble colorlakes. It is furthermore possible to add hygroscopic bodies, for instance glycerine or calcium chloride, which promote the development by retaining in the film or paper a rather large quantity of hygroscopic humidity.

90 Other products may likewise be added, which are destined to modify or ameliorate the properties of the pictures obtained or to increase the stability of the light-sensitive preparation, for instance organic acids. Products, such as thiourea, may also be added in order to preserve the pure whites or lights of the pictures.

95 As a solution for sensitizing paper or films from transparent regenerated cellulose there may be utilized, for instance, an aqueous solution containing 1 per cent of the diazo chloride obtained by diazotizing the hydrochloride of para-amino-diphenyl-amine, 2 per cent of tartaric acid and 8 per cent of glycerine. Generally, there may be used all diazo compounds usual in diazo-type 100 105 110

processes, such, for instance, as diazo compounds of aromatic diamines, amino-acylamines, amino-phenyl-ethers and substitution products thereof. Thus the diazo-compounds of anisidine, dianisidine, aminodiethylaniline, amino-diphenyl-ether or similar products are suitable for the new process.

The paper or film thus treated is exposed to light under a pattern, developed and fixed as follows: A strip of blotting paper or tissue has been impregnated with a 6 per cent alcoholic solution of an aromatic mono- or di-amine capable of coupling with diazo compounds and being volatile in a certain degree, such as alpha-naphthylamine or meta-toluylene-diamine having a considerable vapor tension at ordinary temperature; the said strips have been allowed to dry and a sort of book has been composed therefrom which is placed into a metal envelope. The prints to be developed are placed between the foils of the said book and left therein for a sufficiently long time, for instance, for half an hour in the case of prints produced on the paper prepared as above described. Pictures are obtained which have a blue shade when alpha-naphthylamine has been used, and a violet shade when meta-toluylene-diamine has been employed. According to the diazo compound used and the amine employed for the development there may be obtained the most varied shades varying from red and yellow to black. The shades may furthermore be altered by utilizing two or more different diazo compounds and amine mixtures. The pictures may also be washed or subjected to an after treatment, such as is usual in diazotype printing, for instance with metal salts.

The action of heat and humidity increases the rapidity of the development.

The application of pressure for producing an intimate contact between amine and light-sensitive preparation likewise accelerates the development. If all conditions remain unaltered, the rapidity of the development varies with the nature of the light-sensitive diazo-compound used and the amine applied. For a paper sensitized with the diazotization product of the hydrochloride of para-aminodimethylaniline the duration of development may, for instance, be reduced to 10 minutes or even less.

The vapors of amines serving for the development may, of course, also be produced under other conditions, for instance in a heated vessel containing the amine or an alcoholic solution thereof. It is also possible to carry out a continuous development by utilizing a machine comprising feeding devices for the paper to be developed; the said feeding devices, consisting of cylinders coated with endless tissue or felt which has previously been impregnated with an amine.

Some examples relating to the development of diazo-copies with amines are given below.

#### Examples

1. Cellulose foil is impregnated with a solution containing 1.2 parts by weight of diazodiphenylamine sulphate, 20 parts by volume of glycerine, 1.5 parts by weight of citric acid in 90 parts by volume of water, and on this material copies in the following tints are obtained by the present process:

With m-toluylene diamine bluish violet,  
With  $\alpha$ -naphthylamine yellowish red,  
With m-aminophenol red,  
With dimethyl aniline brownish red,  
75 With o-anisidine reddish.

2. If cellulose foil is impregnated with a solution of 1.2 parts by weight of the zinc chloride double salt of the diazo-compound of p-aminodiethylaniline, 0.8 parts by volume of tartaric acid, and 20 parts by volume of glycol in 80 parts by volume of water, olive green tints can be obtained with m-toluylene diamine and yellowish brown copies with m-aminophenol.

3. A nitrocellulose film provided with a layer of gelatine is impregnated with a solution of 2.5 parts by weight of the zinc chloride double salt of the diazo-compound of p-aminooethylbenzyl-aniline, 0.8 parts by volume of tartaric acid and 10 parts by volume of glycerine in 90 parts by volume of water. After exposing under an original copy and developing by the process described hereinbefore copies in the following tints are obtained:

With m-toluylene diamine violet, 95  
With m-aminophenol brown,  
With mono-ethylaniline brownish,  
With  $\alpha$ -naphthylamine brown.

4. Cellulose foil impregnated with a 1.5 per cent solution of tetrazodianisol gives brownish 100 copies when developed with m-toluylene diamine and brownish violet pictures with  $\alpha$ -naphthylamine.

5. Cellulose hydrate foil is sensitized with a solution consisting of 1 part by weight of diazodiphenylamine sulphate, 1 part by weight of tartaric acid, 1 part by weight of resorcin, 20 parts by weight of glucose and 180 parts by volume of water. On developing by the process hereinbefore described, m-toluylene diamine gives bluish 110 violet copies and m-aminophenol red copies.

I claim:

1. The process of preparing diazotypes which comprises exposing a material sensitized by means of light-sensitive aromatic diazo compounds to light under a pattern and then treating it with the vapors of an aromatic amine capable of coupling with diazo compounds. 115

2. The process of preparing diazotypes which comprises exposing a material sensitized by means of light-sensitive aromatic diazo compounds to light under a pattern and then treating it with a dry support which has been impregnated with a volatile aromatic amine capable of coupling with diazo compounds. 120

3. The process of preparing diazotypes which comprises exposing a material sensitized by means of light-sensitive aromatic diazo compounds to light under a pattern and then treating it with vapors of alpha-naphthylamine. 130

4. The process of preparing diazotypes which comprises exposing a material sensitized by means of light-sensitive aromatic diazo compounds to light under a pattern and then treating it with a dry support which has been impregnated with alpha-naphthylamine. 135

5. The process of preparing diazotypes which comprises exposing a material sensitized by means of light-sensitive aromatic diazo compounds to light under a pattern and then treating it with vapors of meta-toluylenediamine. 140

6. The process of preparing diazotypes which comprises exposing a material sensitized by means of light-sensitive aromatic diazo compounds to light under a pattern and then treating it with a dry support which has been impregnated with meta-toluylenediamine. 145